

July 31, 1945.

L. O. BUXTON

2,380,412

HIGH IODINE VALUE OILS

Filed July 29, 1942

2 Sheets-Sheet 1



FIG. I

INVENTOR

LORAN O. BUXTON

BY *Donald A. Swanson*  
ATTORNEY

July 31, 1945.

L. O. BUXTON

2,380,412

HIGH IODINE VALUE OILS

Filed July 29, 1942

2 Sheets-Sheet 2



FIG. 2

INVENTOR  
LORAN O. BUXTON  
BY  
*Harold A. Swanson*  
ATTORNEY

## UNITED STATES PATENT OFFICE

2,380,412

## HIGH IODINE VALUE OILS

Loran Old Buxton, East Orange, N. J., assignor  
to National Oil Products Company, Harrison,  
N. J., a corporation of New Jersey

Application July 29, 1942, Serial No. 452,775

12 Claims. (Cl. 260—426)

This invention relates to the production of drying oils, more particularly to the production of drying oils for use in paints, varnishes, and similar materials.

For many years linseed oil has been the oil principally used in paints and varnishes to give them their characteristic drying properties. Because of the somewhat erratic fluctuations in the flaxseed crop, the price of linseed oil is quite frequently relatively high. Because of this and other reasons a number of substitutes for linseed oil have been proposed. Vegetable oils such as soybean oil and similar oils have been suggested, but, although they may be used in admixture with linseed oil, they are not satisfactory as they form soft, gummy films. Fish oils may also be used in conjunction with linseed oil, but even though they usually have a much higher iodine value than the vegetable oils and are fairly rapid driers, they also form soft, tacky films and are therefore no more applicable for use alone than are the vegetable oils. Much work has been done along the line of developing new and known but not extensively grown plants for producing drying oils and also along the line of chemical processing of the relatively cheap and available oils in order to produce drying oils, but, as yet, no satisfactory, readily available, economical replacement for linseed oil for use in paints or varnishes has been developed.

It is the object of this invention to provide a process for producing improved drying oils from fish oils.

Another object of this invention is to provide a low cost drying oil to entirely replace linseed oil in paints and varnishes.

Still another object of this invention is to provide an economical, readily available supply of drying oils for paints and varnishes.

Other objects of the invention will in part be obvious and in part appear hereinafter.

Fish oils are composed essentially of a mixture of triglycerides of various higher fatty acids having varying molecular weights and varying degrees of unsaturation. The unsaturated triglycerides in fish oils have, for the most part, a higher molecular weight than the more saturated triglycerides. Contrary to the general belief, I have found that in partially saponifying a fish oil the saturated and slightly unsaturated triglycerides, hereinafter referred to as "saturated glycerides," are selectively saponified, i. e. the saturated and slightly unsaturated triglycerides take precedence over unsaturated triglycerides in order of reaction with alkaline agents. In consequence to the foregoing finding, I have found that excellent drying oils of high iodine value may be produced from oils of fish origin by partially saponifying the same in such a manner that the more saturated glyceride components of the oil are selec-

tively saponified, leaving a large part of the highly unsaturated fatty acid components of the oil esterified with glycerol. That part of the fish oil which has been saponified is then separated from the unsaponified fraction the latter of which has an iodine value substantially higher than the original oil and is characterized by having excellent drying and film-forming properties.

In order to bring about the desired selective saponification, I have found that it is very important that this reaction proceed slowly under controlled conditions. If the reaction is carried out at a rapid rate, as is usually the case, e. g. in soap manufacture, the saponification will not be selective, but instead the more highly unsaturated components of the oil will be saponified as readily as the saturated components. Consequently, even though the fish oil may be only partially saponified if the reaction is carried out at a fairly rapid rate, the portion of the oil which is not saponified will have practically the same degree of unsaturation as the original oil.

I have found that the ester linkages between the more saturated, the shorter chain and the lower molecular weight fatty acids, and glycerol are not as strong as the ester linkages between the highly unsaturated fatty acids and glycerol; consequently, the former are more readily broken and if the conditions of saponification are properly controlled, such linkages are ruptured whereas the linkages between the more highly unsaturated fatty acids and glycerol are not broken. When the saponified saturated fatty acids are removed from the partially saponified mixture, the oil which remains is highly unsaturated and serves as an excellent drying oil. However, if the conditions of saponification are made somewhat more severe the unsaturated fatty acids in some cases split off from the glycerol as readily as the saturated ones, and therefore in such cases the degree of unsaturation of the unsaponified oil, for all practical purposes, will not have been increased whatsoever.

The invention accordingly comprises the several steps and relation of one or more of such steps with respect to each of the others, and the product possessing the features, properties and the relation of elements, which are exemplified in the following detailed disclosure, and the scope of the invention will be indicated in the claims.

In selectively and partially saponifying the fish oil with caustic alkali, the partial saponification may be carried out without the presence of a solvent medium; however, it is preferred that the selective and partial saponification be carried out in the presence of a solvent, preferably a hydrocarbon or halogenated hydrocarbon solvent for the fish oil. Suitable solvents in which fish oils may be selectively and partially saponified include, *inter alia*, ethylene dichloride, methylene

dichloride, trichloroethylene, heptane, hexane, cyclohexane, methyl cyclohexane, etc., or a mixture of two or more of these or other solvents for fish oils which will not dissolve any appreciable amount of water or hydrated alkali metal soap.

The oil is preferably diluted with solvent before adding the saponification agent. When the oil is diluted with solvent for carrying out the selective partial saponification step, the solvent should comprise from 15% to 99% and preferably 25% to 75% based on the weight of the oil.

The selective partial saponification of the fish oil is preferably effected by slowly stirring a suitable alkaline agent such as sodium carbonate, sodium hydroxide, potassium carbonate or potassium hydroxide, aqueous potassium hydroxide usually being preferred, into the solvent-diluted oil, care being taken to insure thorough mixing and to avoid too rapid saponification. Alkali is added in quantities sufficient to saponify 30% to 90% and preferably 40% to 80% of the fish oil being treated. The degree of saponification will be varied considerably depending upon the particular oil treated as well as upon the characteristics desired in the end product.

As a relatively slow rate of saponification appears to be the most favorable for selective saponification of the more saturated fatty acids, I prefer to carry out the saponification at room temperature. In some cases when saponifying at room temperatures (i. e. without supplying heat), it is desirable to employ a saponification catalyst, such as, for example, isopropanol, ethanol, methanol, etc., to aid in bringing about a reaction between the oil and the alkali. This is particularly true when saponifying in the presence of a hydrocarbon or halogenated hydrocarbon solvent. Of course, the rate of saponification may be retarded by reducing the amount of saponification catalyst ordinarily used, when complete saponification is desired, or by not using any at all, also, by using a less concentrated alkali, etc. If desired, saponification inhibitors may be used to retard the rate of reaction; however, that is seldom necessary when the reaction is carried out at room temperature. Also, if desired, the rate of saponification may be retarded by carrying the reaction out at a temperature below room temperature.

In separating the unsaponified portion of the fish oil from the soaps which have been formed, I prefer to extract the partially saponified mass with a hydrocarbon or halogenated hydrocarbon solvent, such as one of the solvents suitable for use in diluting the oil prior to the saponification step, and preferably the same solvent as was used during the saponification step. Before extracting the selectively partially saponified mass with solvent, I prefer to adjust the water content thereof to about 22% to about 26% based on the weight of the soap present in the mass, as usually the separation of the saponified portion from the unsaponified portion is most efficiently accomplished when the moisture content of the soap mass is within this range. Of course, the unsaponified oil may be separated from the soap by other means, e. g., centrifugation, etc., if desired.

Any oil of fish origin may be treated by the process of my invention, e. g. fish body oils and fish liver oils. Among the fish oils which I prefer to treat there may be mentioned sardine oil, shark oil, shark liver oil, herring oil, pilchard oil, menhaden oil, salmon oil, skate oil, sword fish liver oil, cod liver oil, cod oil, ling cod liver oil, halibut liver oil, tuna liver oil, tuna oil, mackerel

liver oil, mackerel oil, sole liver oil, spear fish liver oil, etc. Also, if desired, mixtures of any of these or other fish oils may be treated. The expression "fish oil" is employed herein to connote oils of fish origin, i. e. fish body oils and fish liver oils.

For a fuller understanding of the nature and objects of the invention, reference should be had to the following examples which are given merely to further illustrate the invention and are not to be construed in a limiting sense, all parts given being by weight.

#### Example I

15 200 parts of sardine oil were mixed with 100 parts of ethylene dichloride, 6 parts of 99% isopropanol and 60 parts of 46% aqueous KOH (sufficient to saponify about 80% of the oil). The mixture was then stirred at room temperature for about 20 minutes and the mass left at room temperature over night. The partially saponified mass was then mixed with about 600 parts of additional ethylene dichloride, and the mixture warmed to about 40° C. to coagulate the soaps. 20 The moisture content of the soap was then increased to about 24%, the mixture cooled to about 25° C., and the unsaponified fraction extracted with additional batches of fresh solvent. The extracts were filtered and the solvent removed. 25 The oil thus obtained was light yellow in color, had an iodine value of 216 and dried rapidly on exposure to air to form a firm durable film. The original sardine oil had an iodine value of 186 and on drying formed a soft tacky film.

#### Example II

30 A sample of shark liver oil which had an iodine value of about 184 was treated essentially as described in Example I. The resulting oil had an iodine value of 234 and formed a firm durable film on drying.

#### Example III

35 200 parts of cold pressed sardine oil having an iodine value of 186 were mixed with 100 parts of ethylene dichloride and the mixture agitated for 3 hours at room temperature with 43 parts of 46% NaOH. The mass was allowed to stand at room temperature for about 60 hours. It was then mixed with 600 parts of ethylene dichloride and the water content adjusted to about 24% (based on the weight of the soap). The ethylene dichloride, which contained the major part of the unsaponified portion of the oil, was removed, and the remainder of the oil removed from the 40 soap mass by extracting the mass with additional fresh batches of ethylene dichloride. The extracts were filtered and the solvent removed. A light yellow oil resulted having an iodine value of 208 and characterized by having excellent 45 drying properties.

#### Example IV

50 100 parts of sardine oil were mixed at room temperature with 30 parts of 46% aqueous KOH (sufficient to saponify about 80% of the oil) in the presence of 15 parts of 99% isopropanol. The mixture was relatively solid in about 6 minutes, and the temperature of the mixture had increased to 51° C. The partially saponified mass 55 was allowed to stand overnight, and the unsaponified portion then extracted therefrom with ethylene dichloride as described in Example I. The oil was light yellow in color and the iodine value was 210 as compared to 183 for the original oil.

**Example V**

A sample of the same sardine oil as was used in Example IV was treated in essentially the same manner as in Example IV, the principal difference being that in this case 40% aqueous KOH was used instead of 46%. It was necessary to continue stirring for 11 minutes before the mass became solid enough to hold its shape. At that time the temperature was only 37° C. as compared to 51° C. in Example IV which indicates that with the less concentrated caustic, the saponification proceeds at a slower rate. Although the same yield of oil was obtained in both examples, the iodine value of the oil obtained in this case was 222 as compared to 210 in Example IV. This very clearly illustrates that selective saponification is obtained by varying the saponification conditions, i. e. the milder the conditions, the more selective the saponification.

**Example VI**

100 parts of shark liver oil having an iodine value of 175 were mixed with 50 parts of ethylene dichloride and 1 part of 99% isopropanol. While stirring, sufficient 46% KOH (22 parts) to saponify about 55% of the oil was added and the mixture stirred for 5 hours. The solid soap was kept at room temperature overnight and then treated further in the usual manner to separate the unsaponified oil from the partially saponified mass. The resulting oil was light yellow in color, had an iodine value of 206 and formed a firm durable film on drying.

**Example VII**

100 parts of sardine oil having an iodine value of 183 were mixed with 50 parts of ethylene dichloride and 3 parts of 99% isopropanol and, while stirring, sufficient 46% aqueous KOH (29.5 parts) to saponify about 70% of the oil was added. The mixture was treated further much the same as in the above examples. A light colored oil having an iodine value of 216 and having excellent drying properties was obtained.

**Example VIII**

100 parts of herring oil were mixed with 50 parts of ethylene dichloride, 3 parts of 99% isopropanol and, while stirring, sufficient 46% aqueous KOH (31 parts) to saponify about 80% of the oil was added. The mass was then treated further much the same as in the above examples. The oil which was obtained had an iodine value of 170 as compared to 135 for the original oil.

**Example IX**

This example was carried out in exactly the same manner as Example VIII, the only difference being that a sample of cod liver oil having an iodine value of 149 was used in place of herring oil. A very good drying oil having an iodine value of 185 was obtained.

The following table summarizes some of the many experiments which were carried out on various fish oils and fish liver oils under varying reaction conditions and with varying degrees of saponification. Unless otherwise specified the saponifying agent employed was commercial, concentrated potassium hydroxide, i. e. 46% aqueous potassium hydroxide; also unless otherwise stated, the reaction was carried out with mild agitation of the reaction mixture. The word "solvent" is used in the table to indicate that the reaction was carried out in the presence

5 of ethylene dichloride, employing 50 parts of ethylene dichloride to every 100 parts of oil. The word "catalyst" as used in the table refers to isopropanol and the percentage given is based on the weight of the oil. All of the saponification reactions were carried out at room temperature, i. e. without supplying any extraneous heat.

**Table I**

| 10 | Oil               | Saponification | Conditions                                          | Iodine value |             |
|----|-------------------|----------------|-----------------------------------------------------|--------------|-------------|
|    |                   |                |                                                     | Orig-inal    | End product |
| 15 |                   | Per cent.      |                                                     |              |             |
|    | Sardine No. 1     | 79             | Solvent 3% catalyst                                 | 178          | 216         |
|    | Sardine No. 2     | 75             | do                                                  | 183          | 215         |
|    | Do                | 54             | do                                                  | 183          | 201         |
|    | Sardine No. 3     | 76             | do                                                  | 181          | 219         |
|    | Sardine No. 4     | 77             | Solvent 3% catalyst<br>medium stirring.             | 184          | 223         |
| 20 | Do                | 77             | Solvent 3% catalyst<br>slow stirring.               | 184          | 230         |
|    | Do                | 80             | No solvent 3% cata-<br>lyst dilute alkali<br>(40%). | 184          | 222         |
|    | Do                | 80             | No solvent 1.5%<br>catalyst.                        | 184          | 210         |
| 25 | Herring           | 82             | Solvent 3% catalyst                                 | 135          | 169         |
|    | Cod liver         | 80             | do                                                  | 149          | 186         |
|    | Shark liver No. 1 | 80             | do                                                  | 183          | 234         |
|    | Shark liver No. 2 | 74             | do                                                  | 176          | 216         |
|    | Do                | 51             | do                                                  | 176          | 203         |
|    | Do                | 25             | do                                                  | 176          | 184         |
|    | Shark liver No. 3 | 43             | do                                                  | 167          | 190         |
| 30 | Shark liver No. 4 | 71             | No solvent 3% cata-<br>lyst.                        | 178          | 212         |
|    | Do                | 43             | do                                                  | 178          | 191         |
|    | Tuna liver        | 37             | Solvent 3% catalyst                                 | 149          | 162         |
|    | Halibut liver     | 28             | do                                                  | 137          | 151         |
|    | Menhaden No. 1    | 83             | do                                                  | 171          | 212         |
|    | Do                | 51             | do                                                  | 171          | 192         |

35 In the accompanying drawings Figure 1 comprises three curves depicting the increase in iodine value of three oils when subjected to varying degrees of partial saponification; Figure 2 comprises four curves illustrating the increase in iodine value when a shark liver oil was subjected to various methods of partial saponification.

40 In Figure 1, curves 1, 2 and 3 represent the increase in iodine value of shark liver oil, sardine oil and menhaden oil, respectively, when subjected to varying degrees of saponification. In each case 100 parts of oil containing 50 parts of ethylene dichloride and 3 parts of isopropanol were reacted to yield the indicated degree of saponification. The points plotted on the graph constituting Figure 1 bear the values indicated in the following table:

| 55 | Oil                   | Saponifi-<br>cation | Iodine<br>value |  |
|----|-----------------------|---------------------|-----------------|--|
|    |                       |                     | Per cent.       |  |
|    | Shark liver (curve 1) | 00.0                | 178.0           |  |
|    | Shark liver           | 28.5                | 184.6           |  |
|    | Do                    | 43.9                | 192.3           |  |
|    | Do                    | 58.0                | 203.3           |  |
|    | Do                    | 71.4                | 212.5           |  |
|    | Do                    | 86.1                | 223.0           |  |
|    | Sardine (curve 2)     | 00.0                | 184.4           |  |
|    | Do                    | 18.6                | 188.5           |  |
|    | Do                    | 28.0                | 190.3           |  |
|    | Do                    | 41.2                | 193.8           |  |
|    | Do                    | 58.7                | 201.9           |  |
|    | Do                    | 71.8                | 210.5           |  |
|    | Do                    | 80.9                | 217.5           |  |
|    | Do                    | 90.0                | 236.5           |  |
|    | Menhaden (curve 3)    | 00.0                | 172.5           |  |
|    | Menhaden              | 31.4                | 178.0           |  |
|    | Do                    | 52.9                | 188.5           |  |
|    | Do                    | 73.6                | 196.0           |  |
|    | Do                    | 83.4                | 210.0           |  |
|    | Do                    | 90.9                | 231.0           |  |

70 In Figure 2, curves 1, 2, 3 and 4 all represent a shark liver oil subjected to varying degrees of

saponification under four separate sets of conditions. The oil represented by curve 1 was partially saponified by caustic potash without the presence of either solvent or catalyst. The oil represented by curve 2 was partially saponified without the presence of solvent, but in the presence of 0.75% isopropanol. The oil represented by curve 3 was partially saponified without the presence of solvent, but in the presence of 3.0% isopropanol. The oil represented by curve 4 contained 50% ethylene dichloride and 3.0% isopropanol, based on the weight of the oil, upon partial saponification. The points plotted on the graph constituting Figure 2 bear the values set forth in the following table:

*Shark liver oil having original iodine value of 175.9*

| Conditions                 | Saponification | Iodine value |
|----------------------------|----------------|--------------|
| No catalyst or solvent     | Per cent       |              |
| Do.                        | 31.4           | 188.0        |
| Do.                        | 52.2           | 204.5        |
| Do.                        | 67.5           | 213.5        |
| Do.                        | 91.0           | 207.3        |
| No solvent, 0.75% catalyst | 30.4           | 191.7        |
| Do.                        | 51.3           | 201.3        |
| Do.                        | 92.2           | 199.7        |
| No solvent, 3.0% catalyst  | 30.3           | 188.2        |
| Do.                        | 50.4           | 195.1        |
| Do.                        | 66.0           | 190.1        |
| Do.                        | 81.7           | 190.9        |
| Solvent and 3% catalyst    | 29.3           | 187.7        |
| Do.                        | 54.3           | 203.2        |
| Do.                        | 63.2           | 214.6        |
| Do.                        | 86.9           | 223.0        |

The curves shown in Figure 2 clearly reveal the superior results obtained by carrying out the partial selective saponification in the presence of a solvent for the oil along with a small quantity of catalyst. In carrying out the process of the invention on a commercial scale it is advisable to perform preliminary experiments on the particular fish oil to be processed in order to determine the optimum conditions. Fish oils vary considerably in their properties and characteristics and in their reaction or behavior when treated according to the process of this invention. It has been found that different batches of the same species of fish oil likewise vary. For example, different batches of shark liver oil were employed in the experiments depicted by curve 1 of Figure 1 and curve 4 of Figure 2. The differences in the results obtained are clearly indicated by a comparison of these two curves. Hence, it is important to determine beforehand the behavior of any given fish oil when treated according to the process of the invention.

In practically every case, the drying oil obtained was much lighter in color than the original oil, usually being light yellow. This is another important advantage of my process as light colored oils are much preferred by the industry. Furthermore, the oils produced have lost the major portion of the fishy odor of the original oils, and thus are highly satisfactory in that respect. Also these oils are completely devoid of free fatty acids. The products of my invention are quite fluid and have low cloud and pour points because of the removal of the more saturated components therefrom.

Drying oils are in many cases "bodied" before being used, either by heating at atmospheric pressure, heating under a vacuum, blowing air through the oil, etc. Because of their highly un-

saturated character, my drying oils are much more adaptable to being "bodied" than are many of the natural drying oils. Furthermore, because of their highly unsaturated character, my drying oils may be readily sulfonated yielding products of high SO<sub>3</sub> content.

The partial saponification of fish oils in addition to selectively saponifying the more saturated components thereof also destroys the major portion of any natural antioxidants that may be present in the oil. Consequently, the rate of drying of the oil is still further increased. Thus, by eliminating the majority of the more saturated components of the oil and the major portion of the natural antioxidants therein, an oil having a very high iodine value and rapid drying qualities is obtained. If desired, the iodine value of the unsaponified portion of the partially saponified oil which is obtained may be further stepped up by solvent fractionation or other conventional means.

The soaps which are formed as by-products of the process of my invention may be utilized for various purposes, e. g. they may be split by acid hydrolysis and the fatty acids recovered and used as such or for other purposes for which they are adapted. Since the major part of the fatty acids in those soaps are much more highly saturated than is usually the case with fish oil soaps, the soaps which are produced as by-products of my invention are in many cases more useful than the ordinary fish oil soaps. The high iodine value fraction produced in accordance with this invention may be hydrolyzed to produce highly unsaturated fatty acids of high molecular weight. Thus, it may be seen that this invention affords a means of recovering from fish oils the higher molecular weight fatty acids, i. e. acids containing 20 or more carbon atoms.

Since certain changes in carrying out the above process and certain modifications in the composition which embody the invention may be made without departing from its scope, it is intended that all matter contained in the above description shall be interpreted as illustrative and not in a limiting sense.

Having described my invention, what I claim as new and desire to secure by Letters Patent is:

1. A process of producing high iodine value oils from fish oils which comprises selectively saponifying 30% to 90% of a fish oil by means of an alkali to split saturated glycerides and separating the unsaponified fraction from the resulting soap mass.

2. A process of producing high iodine value oils from fish oils which comprises admixing a fish oil with a lesser quantity of a water-immiscible organic solvent therefor, saponifying 30% to 90% of the fish oil by means of an alkali and separating the unsaponified fraction from the saponified mass.

3. A process of producing high iodine value oils from fish oils which comprises admixing a fish oil with a lesser quantity of a hydrocarbon solvent therefor, saponifying 30% to 90% of the fish oil by means of an alkali and separating the unsaponified fraction from the saponified mass.

4. A process of producing high iodine value oils from fish oils which comprises admixing a fish oil with a lesser quantity of a halogenated hydrocarbon solvent therefor, saponifying 30% to 90% of the fish oil by means of an alkali and separating the unsaponified fraction from the saponified mass.

5. A process of producing high iodine value oils

from fish oils which comprises admixing a fish oil with a lesser quantity of ethylene dichloride, saponifying 40% to 80% of the fish oil by means of an alkali and separating the unsaponified fraction from the saponified mass.

6. A process of producing high iodine value oils from fish oils which comprises admixing a fish oil with a lesser quantity of a hydrocarbon solvent therefor, saponifying 30% to 90% of the fish oil by means of an alkali in the presence of a saponifying catalyst and separating the unsaponified fraction from the saponified mass.

7. A process of producing high iodine value oils from fish oils which comprises admixing a fish oil with a lesser quantity of ethylene dichloride, saponifying 40% to 80% of the fish oil by means of an alkali in the presence of a small quantity of isopropanol and separating the unsaponified fraction from the saponified mass.

8. A process of producing high iodine value oils from fish oils which comprises admixing in the presence of an alcoholic saponification catalyst a fish oil having a lesser quantity of a water-immiscible organic solvent dissolved therein with a quantity of alkali sufficient to saponify 30% to 90% of the fish oil, stirring the mass to form a super-solvent emulsion, breaking the emulsion by means of heat to flocculate the soap, adding a further quantity of water-immiscible organic solvent to cause complete separation of the flocculated soap particles and separating the solvent solution of the unsaponified high iodine value oil from the soap particles.

9. A process of producing high iodine value oils from fish oils which comprises admixing in the presence of an alcoholic saponification catalyst a fish oil having a lesser quantity of ethylene dichloride dissolved therein with a quantity of alkali sufficient to saponify 30% to 90% of the fish oil, stirring the mass to form a super-solvent emulsion, breaking the emulsion by means of heat to flocculate the soap, adding a further quantity of ethylene dichloride to cause complete separa-

tion of the flocculated soap particles and separating the solvent solution of the unsaponified high iodine value oil from the soap particles.

10. A process of producing high iodine value oils from fish oils which comprises admixing in the presence of isopropanol a fish oil having a lesser quantity of ethylene dichloride dissolved therein with a quantity of alkali sufficient to saponify 40% to 80% of the fish oil, stirring the mass to form a super-solvent emulsion, breaking the emulsion by means of heat to flocculate the soap, adding a further quantity of ethylene dichloride to cause complete separation of the flocculated soap particles and separating the solvent solution of the unsaponified high iodine value oil from the soap particles.

11. A process of producing high iodine value oils from fish oils which comprises admixing in the presence of isopropanol a sardine oil having a lesser quantity of ethylene dichloride dissolved therein with a quantity of alkali sufficient to saponify 40% to 80% of the said oil, stirring the mass to form a super-solvent emulsion, breaking the emulsion by means of heat to flocculate the soap, adding a further quantity of ethylene dichloride to cause complete separation of the flocculated soap particles and separating the solvent solution of the unsaponified high iodine value oil from the soap particles.

12. A process of producing high iodine value oils from fish oils which comprises admixing in the presence of isopropanol menhaden oil having a lesser quantity of ethylene dichloride dissolved therein with a quantity of alkali sufficient to saponify 40% to 80% of the said oil, stirring the mass to form a super-solvent emulsion, breaking the emulsion by means of heat to flocculate the soap, adding a further quantity of ethylene dichloride to cause complete separation of the flocculated soap particles and separating the solvent solution of the unsaponified high iodine value oil from the soap particles.

LORAN OID BUXTON.